

March 17, 1931.

W. F. DETWILER

1,797,053

METHOD OF ROLLING

Filed Dec. 14, 1927

2 Sheets-Sheet 1



INVENTOR  
William F. Detwiler  
By Green and McAlister  
His Attorneys.

March 17, 1931.

W. F. DETWILER

1,797,053

METHOD OF ROLLING

Filed Dec. 14, 1927

2 Sheets-Sheet 2

Fig. 2. 20



INVENTOR  
William F. Detwiler  
By Green and Galster  
His Attorneys

## UNITED STATES PATENT OFFICE

WILLIAM F. DETWILER, OF TARENTUM, PENNSYLVANIA, ASSIGNOR TO ALLEGHENY STEEL COMPANY, OF BRACKENRIDGE, PENNSYLVANIA, A CORPORATION OF PENNSYLVANIA

## METHOD OF ROLLING

Application filed December 14, 1927. Serial No. 239,905.

This invention relates broadly to the manufacture of metal sheets and more particularly to the manufacture of "full finished" sheets such as low carbon steel sheets commonly referred to as automobile and furniture sheets because of their highly finished surfaces and suitability for deep stamping operations.

The utility of the present invention is not limited, however, with respect to the analysis of the sheets produced nor to the uses to which such sheets are to be put.

The standard or ordinary method of producing sheets comprises a long series of steps in which the material is alternately heated and rolled and in which the rolling operations are further involved by matching, pairing, doubling, shearing and opening.

Cunningham Patent No. 1,536,663 of May 5, 1925 sets forth a method of rolling sheets in which the standard or ordinary methods are modified by substituting certain cold rolling operations for some of the hot rolling operations. It may be said that this patent contemplates a reduction by hot rolling and a material reduction by cold rolling so carried forward that the sheets when annealed are free from Stead's brittleness. Caugherty and Hookey Patent No. 1,536,660 of the same date sets forth a modification of the Cunningham method in which a somewhat greater reduction is made during the cold rolling operation with a resultant saving in cost.

While I follow to some extent the methods set forth by the above mentioned patents, in that I accomplish a material reduction by both hot and cold rolling and produce sheets free from Stead's brittleness, my improved method differs from the methods of these patents as well as from the standard or ordinary methods of rolling sheets in that I eliminate difficult and expensive hot rolling operations, which to some extent characterize all these methods, and I in fact eliminate all hot rolling operations which specifically characterize heretofore known methods of rolling sheets.

In the accompanying drawings, I have shown more or less diagrammatically for

purposes of illustration only, the successive steps utilized in carrying out the method of this invention, it being understood that the drawings do not define the limits of the invention as changes in the construction of the different elements of equipment and in the operation thereof may be made in many instances without departing either from the spirit of the invention or from the scope of my broader claims.

Figure 1 is a diagrammatic view illustrating steps or operations which may be successively employed in carrying forward my invention. These steps or operations are indicated by diagrammatic views of apparatus for performing them.

Fig. 2 is a diagrammatic view of one form of four-high mill and accessory equipment utilized for the obtaining of certain desirable results in accordance with the present method.

In practicing the present invention, I may start with an ingot 2 heated to the desired temperature and subject this ingot to a rolling operation in one or more suitable mills 3 for producing a billet or strip 4 having the desired width and thickness, with the length thereof dependent upon the original size of ingot 2 and the amount of reduction to which the ingot is subjected in the rolling operation. This strip or billet 4 may be subjected to the action of shears 5 for the production of slabs 6 of the desired dimensions.

The slabs are of such dimensions as to be readily handled and are subjected to a heating operation in a suitable furnace 7; the slabs preferably but not necessarily, passing therethrough in substantially flat position as indicated. After being raised to the desired temperature in furnace 7, these slabs are subjected to an edge rolling operation in an edging roll pass 8 for the purpose of breaking the scale therefrom. Without reheating, and with the scale effectively removed by the scale breaker, the slabs are subjected to a further rolling operation in either a two-high reversible or three-high continuous mill 9 suitable for transforming the slabs into skelp 10.

The skelp as produced is piled in any de-

sired manner into a pile or stack 11 so that the heat stored in the mass of piled skelp is effective for the self annealing of the material. After the annealing has been completed, the skelp may be sheared cold by a shear 12 into lengths 14, which for the purposes of this application, I term skelp plates. These skelp plates preferably have a length substantially equal to the width of the sheets to be produced therefrom. These skelp plates are then preferably subjected to a pickling operation in a bath 15 to remove all scale therefrom and to provide clean surfaces. These pickled skelp plates may thereafter be arranged in piles 16 or otherwise conveniently arranged for subsequent use.

The passes of the skelp mill 9 are preferably formed so as to scarf the skelp along both edges in order that either long edge of the skelp plates may be readily entered in the passes of the cold roll mills. One or both long edges of the skelp or skelp plates may be beveled in any manner other than by scarfing if desired, but I find that the cheapest way of beveling these edges is by scarfing the skelp during its formation.

The pickled and cold skelp plates having their long edges beveled are now subjected to a cold rolling operation comprising one or more passes in either the same mill or in a series of similar mills.

Before the skelp plates are entered in the first cold roll pass, they are subjected to a cold flattening pass in a mill 16.

When making low carbon steel sheets suitable for deep stamping operations, it is necessary, in order to obtain sheets that are free from Stead's brittleness after final annealing, to subject the sheets or rather the material from which the sheets are being made, to a strain which is at least equal to the strain to which low carbon steel is subjected when it is given about a 10% cold reduction.

The cold rolling of the skelp plates into finished sheets in accordance with this invention is preferably carried out in a series of four-high mills 17 of which any desired number may be provided and I have found that the strain above referred to for producing low carbon steel sheets free from Stead's brittleness after final anneal, may, if desired, be given to the skelp plates in the first cold roll pass and I have found that in order to be sure that the material is subjected to this strain, it is desirable to obtain this strain in the first cold roll pass by effecting about a 10% reduction.

In practicing this invention, I have found that in order to obtain the best results, it is necessary to control the contour of the passes formed by the reducing or work rolls 18 of the four-high mills.

Reducing rolls because of heating due to work and friction during rolling tend to distort or puff as it is ordinarily termed, and con-

sequently in puffing, change the shape or contour of the pass formed thereby. I have found that I am able to overcome any tendency of the reducing rolls 18 to puff or distort by controlling their temperature, and that therefore I am able to accurately control the contour of the passes through these reducing rolls.

I have found that the contour of the reducing passes can be maintained constant if the temperature of the reducing rolls is maintained constant and I have found that this can be satisfactorily done by making the reducing rolls hollow and causing sufficient temperature controlling medium to flow therethrough.

I preferably use water as the temperature controlling medium and control its flow by means of valves as will be readily understood. In some instances where extremely cold water is desirable and is not available, or when the water supply is limited, I find it advantageous to cool the water by passing it through a refrigerating device before it is delivered into the hollow reducing rolls.

The water may enter one end of the rolls and leave at the other end, or one end of the rolls may be plugged and the water conveyed by a pipe into the rolls to a point adjacent the plugged end and then allowed to flow out through the open end around said pipe.

Inasmuch as it is not feasible during rolling to stop the mill or mills and actually measure the temperature of the reducing rolls, I preferably provide means for giving a visible and continuous check on the temperature of such rolls. I preferably accomplish this in the manner disclosed in Figure 2 of the drawings, by utilizing a plurality of gauges 19, which are secured to a rigid bar 20, supported independently of the mill housings 21, by suitable standards 22. By supporting the bar 20 independently of the mill housings, it is not subjected to their deflections. A portion 23 of each of the gauges continuously bears against the surface of one of the backing rolls, preferably in the plane which includes the roll axes, so as to visibly indicate any deflections in such backing roll.

It will be apparent to those skilled in the art, that should the temperature of the work or reducing rolls increase, they will undergo an expansion incident to that temperature increase, which, in turn, is reflected in the deflection of the backing rolls. This will be immediately indicated by the indicating gauges 19, and may be used by the operator, as a basis for determining the condition of the roll pass. Gauges 19 visibly indicate when changes in the contour of the roll passes occur.

By observing these gauges, the operator is advised when to vary the amount or temperature of the water or other cooling medium, circulating through the reducing rolls; in-

creasing the amount, or lowering the temperature, of the cooling medium as the temperature of the reducing rolls increases, and decreasing the amount and increasing the temperature as the opposite condition manifests itself.

The constant indication of the temperature conditions of the reducing rolls is extremely important, facilitating as it does, the maintenance of the desired pass contour.

Because of the fact that I prevent puffing of the reducing rolls of the cold roll mills by flowing cooling medium through the same, I dress these reducing rolls so as to provide a convexity along the line of rolling sufficient to compensate for the spring of the rolls during the rolling operation.

For example, I have found that it is feasible to allow the reducing rolls to spring during rolling .005 of an inch. I have also found that it is possible by means of backing rolls of my construction to limit this spring to .005 of an inch and I therefore dress the reducing rolls so as to provide a convexity along the line of rolling of .005 of an inch, thus insuring a parallel sided or flat rolling pass.

With indicating means of the type herein diagrammatically disclosed, and made the subject of my co-pending application Serial No. 239,904, filed by me on December 14, 1927, the spring of the backing rolls is visibly and continuously indicated, thus constantly advising the operator as to whether or not the desired contour of the working pass is being maintained.

The initial setting of the rolls may be obtained by screw down mechanism 25 of any desired construction and effective against the roll neck bearings. These bearings may be of any desired construction, but I preferably use bearings of the tapered roller type.

I have found that the amount of roll spring of the backing rolls may be reduced to a comparatively small percentage of that heretofore considered as the minimum for four-high mills, by utilizing fillets 26 connecting the roll bodies and necks, and bearing (with respect to radius of curvature) a definite relation to the diameter of the rolls.

In accordance with the present invention, this radius of curvature is equal to at least three per cent of the diameter of the rolls, and preferably considerably in excess of that and up to six per cent. With a 30 inch roll diameter a radius of curvature for the fillets of one and one-half inch has been found to decrease the roll spring under rolling operations from approximately .060 of an inch to .005 of an inch with the same pressure exerted by the screw down mechanism. These fillets, by reducing the roll spring enable me to control the contour of the pass during rolling more accurately than has heretofore been possible.

The cold rolled sheets after leaving the last

stand of rolls may be trimmed and squared by trimming shear 27. After this operation the sheets may be annealed in accordance with standard practice, either by a box anneal or an open anneal 28, after which they may be 70 smooth rolled in a suitable mill 29, and then leveled and smoothed in a suitable leveler 30,

Inasmuch as the skelp plates are delivered to the cold roll mills with clean surfaces provided by the edging pass and the pickling 75 operation in bath 15, these mills are effective in producing extremely smooth and highly finished sheets, which is not the case with any hot rolling method in the presence of the scale incident to the temperatures employed in such rolling.

I have found that by reversing the material end for end between successive cold roll passes, or at least between certain of such passes, a more nearly uniform product with 85 respect to contour is provided, the reversal prevents extreme irregularities or so-called fish tails.

At times, I find it desirable to subject the material in its progress through the cold roll 90 passes to one or more cross rolling operations for the purpose of improving the physical structure of the sheets.

It will be obvious to those skilled in the art that the present invention does away 95 with all surface marring incident to hot rolling, and it enables a more rapid production of full or highly finished sheets than has heretofore been possible. It also reduces the cost of such sheets.

This invention also provides a method of making individual sheets as distinguished from strip sheets without the necessity of carrying out the difficult steps of pair heating followed by the matching, rolling, re-heating, rematching, doubling, and the like 105 incident to standard sheet mill practice.

Other advantages arise from the cold rolling of skelp plates having surfaces which are free from scale and otherwise clean and which are maintained in clean condition 110 during all of the rolling operations from such plates to finished sheets.

Still further advantages of the invention arise from the use of four-high mills in cold rolling; from the control of the spring of the backing rolls of such mills; from the relationship maintained between the backing roll spring and the convexity of the reducing rolls; from the control and maintenance of 120 the desired temperature conditions in the reducing rolls; from the indication of the temperature conditions and roll spring during rolling, and from the control of the characteristics of the finished sheets by the strain 125 to which the material thereof is subjected in the cold rolling passes.

Still further advantages are obtained by the utilization of the scale breaker prior to the formation of skelp from which the skelp 130

plates are produced whereby said plates, prior to pickling, have surfaces which are smoother than would be obtainable during rolling if any scale were present; from the 5 scarfing of the skelp plates and from the flattening of such plates prior to their entrance in the cold roll passes.

This invention provides a method by means of which plates sheared or otherwise formed 10 from skelp are individually cold rolled into finished sheets. The method is extremely flexible and allows individual treatment of each sheet in its progress through the cold roll passes.

15 What I claim as new and desire to secure by Letters Patent is:—

1. The method of rolling sheets, which consists in hot rolling slabs, in cutting said slabs into suitable lengths, in edging such lengths 20 to remove the scale, in rolling such scale free lengths into skelp, in cutting the skelp into lengths substantially equal to the width of the sheets to be produced, in picking the scale from such lengths, then in cold rolling such 25 scale free lengths into finished sheets and then in annealing such sheets.

2. The method of rolling sheets, which consists in hot rolling slabs, in cutting said slabs into suitable lengths, in edging such lengths to 30 remove the scale, in rolling such scale free lengths into skelp, in cutting the skelp into lengths substantially equal to the width of the sheets to be produced, in pickling the scale from such lengths, then in cold rolling such 35 scale free lengths into finished sheets and then in box annealing such sheets.

3. The method of making sheets, which consists in forming scarfed skelp, in hot rolling said scarfed skelp, in shearing the skelp 40 into skelp plates, in pickling said plates to remove the scale, then in feeding a scarfed edge of such plates to cold rolls and in cold rolling the same into finished sheets and then in annealing such sheets.

45 4. The method of making sheets, which consists in forming scarfed skelp, in hot rolling said scarfed skelp, in shearing such skelp into skelp plates, in pickling the scale from such plates then feeding a scarfed edge of 50 such plates to cold rolls and in cold rolling the same into finished sheets and then in annealing such sheets, the drafts during cold rolling being such that the material is given a strain at least equal to that given low carbon 55 steel when it is subjected to about a 10% cold reduction.

5. The method of making sheets, which consists in forming scarfed skelp, in hot rolling said scarfed skelp, in shearing such skelp 60 into skelp plates, in pickling the scale from such plates then in feeding a scarfed edge of such plates to cold rolls and in cold rolling the same into finished sheets and then in annealing such sheets, the reduction in the 65 first cold roll pass being equal to about 10%.

6. The method of making sheets, which consists in hot rolling to form skelp, in self annealing the skelp, in shearing the annealed skelp into skelp plates, in pickling such plates, in cold rolling such pickled plates into finished sheets and then in annealing such sheets.

7. The method of making sheets, which consists in hot rolling to form skelp, in collecting a mass of such skelp and allowing the same to self anneal, in shearing the annealed skelp into skelp plates, in pickling such plates, in cold rolling such pickled plates into finished sheets and then in annealing such sheets.

8. The method of making sheets, which consists in hot rolling to form skelp, in annealing the skelp, in shearing the annealed skelp into skelp plates, in pickling such plates, in cold rolling such pickled plates into finished sheets and then in annealing such sheets.

9. The method of making sheets, which consists in reducing an ingot to billet form, in shearing the billets into slabs, in heating the slabs, in edging the slabs to remove the scale, in rolling the slabs into skelp, in annealing the skelp, in shearing the skelp into skelp plates of a length substantially equal to the width of the sheets to be produced, in pickling such plates, in flattening the same, then in cold rolling the flattened plates to the length and gauge of the finished sheets and then in annealing such sheets.

10. The method of making sheets, which consists in reducing an ingot to billet form, in shearing the billets into slabs, in heating the slabs, in edging the slabs to remove the scale, in rolling the slabs into scarfed skelp, in annealing the skelp, in shearing the skelp into skelp plates of a length substantially equal to the width of the sheets to be produced, in pickling such plates, in flattening the same, then in entering a scarfed edge of such plates to cold rolls and in cold rolling the flattened plates to the length and gauge of the finished sheets and then in annealing such sheets.

11. The method of making sheets, which consists in reducing an ingot to billet form, in shearing the billets into slabs, in heating the slabs, in edging the slabs to remove the scale, in rolling the slabs into skelp and scarfing the skelp, in annealing the skelp, in shearing the skelp into skelp plates of a length substantially equal to the width of the sheets to be produced, in pickling such plates, in flattening the same, then in entering a scarfed edge of such plates in cold rolls and in cold rolling the flattened plates to the length and gauge of the finished sheets and then in annealing such sheets.

12. The method of making sheets, which consists in rolling to form skelp, in annealing the skelp, in shearing the skelp into skelp

plates of a length substantially equal to the width of the sheets to be produced, in pickling the scale from such plates, then in cold rolling such pickled plates into finished sheets through a succession of cold roll passes and then in annealing such sheets, the material between two or more of such cold roll passes being turned end for end.

13. The method of making sheets, which consists in rolling to form skelp, in annealing the skelp, in shearing the skelp into skelp plates of a length substantially equal to the width of the sheets to be produced, in pickling the scales from such plates, then in cold rolling such pickled plates into finished sheets through a succession of cold roll passes and then in annealing such sheets, the material between two or more of such cold roll passes being turned to effect cross rolling thereof.

14. The method of making sheets, which consists in hot rolling to form skelp, in annealing the skelp, in shearing the same into skelp plates, in pickling the scale from such plates and then in cold rolling such pickled plates to the length and gauge of the finished sheets through a succession of cold roll passes in which the pass contours are maintained constant by maintaining the temperature of the reducing rolls constant by flowing a temperature controlling medium through such rolls.

15. The method of making sheets, which consists in hot rolling to form skelp, in annealing the skelp, in shearing the same into skelp plates, in pickling the scale from such plates and then in cold rolling such pickled plates to the length and gauge of the finished sheets through a succession of cold roll passes, maintaining said cold roll passes at constant temperature and controlling the spring of said rolls with the aid of backing rolls.

16. The method of making sheets, which consists in hot rolling to form skelp, in annealing the skelp, in shearing the same into skelp plates, in pickling the scale from such plates, then in cold rolling such pickled plates to the length and gauge of the finished sheets through a succession of cold roll passes maintained at constant temperature and in which the temperature of the reducing rolls is controlled by flowing a temperature controlling medium therethrough, in continuously checking the temperature conditions of such rolls during rolling and in varying the flow of the temperature controlling medium in accordance with such check.

17. The method of making full finished low carbon steel sheets free from Stead's brittleness, which consists in hot rolling slabs to form skelp, in cutting the same into relatively short lengths, in pickling such lengths then in cold rolling the pickled lengths through successive roll passes into

sheets of the length and gauge desired and then in annealing the sheets; the drafts during cold rolling being so controlled that the material is given a strain at least equal to that given low carbon steel when it is subjected to about a 10% cold reduction in a single pass.

18. The method of making sheets, which consists in roll reducing an ingot to form skelp, in self annealing the skelp, in cold shearing the skelp into plates, in pickling the scale from such plates, in cold rolling such plates to the length and gauge desired in the finished sheets, then in annealing the sheets; said cold reduction being accomplished by rolls forming a succession of passes in the first of which a reduction of about 10% is obtained, in reducing the roll spring in such passes by opposing the vertical thrust of the reducing rolls by backing rolls, in visibly indicating changes in temperature in the reducing rolls and in controlling the temperature of the reducing rolls in accordance with said indications by flowing a temperature regulating medium through such rolls.

19. The method of making steel sheets comprising the following steps in substantially the order named: reducing an ingot of steel to form a strip, shearing the strip to form slabs of pre-determined size, heating said slabs by passing them through a furnace of predetermined heat, edge rolling and scarfing said slabs, rolling said scarfed slabs to form skelp, self-annealing said skelp, shearing said scarfed skelp to form skelp plates, pickling said plates, flattening the same, entering a scarfed edge of such plates between cold rolls and plurally cold rolling said plates to pre-determined size, the conditions of cold rolling being mechanically controlled through temperature control, trimming said sheets, annealing them, and finally smoothing and leveling the same.

In testimony whereof, I have hereunto subscribed my name this 10th day of December, 1927.

W. F. DETWILER.

115

120

125

136